

3,632,509

### ELECTRIC CONTACT GREASE

Akira Inami, Hirakata-shi, Osaka-fu, Sankichi Shida, Nara-shi, and Mikio Haga, Osaka-fu, Japan, assignors to Matsushita Electric Industrial Co., Ltd., Kadoma, Osaka, Japan

No Drawing. Filed Jan. 9, 1970, Ser. No. 1,893  
Claims priority, application Japan, June 11, 1969,

44/47,059

Int. Cl. C10m 5/16, 5/18

U.S. Cl. 252—33.3

4 Claims

### ABSTRACT OF THE DISCLOSURE

An improved contact grease is provided. The grease consists essentially of

- (a) a major amount of paraffinic mineral oil;
- (b) 10 to 20 percent by weight of, as a thickening agent, a mixture of metallic soaps, said mixture of metallic soaps consists essentially of
  - (i) 40 to 65 percent by weight of barium soap;
  - (ii) 25 to 40 percent by weight of lithium soap and
  - (iii) 10 to 20 percent by weight of aluminum soap;
- (c) 7 to 15 percent by weight of at least one member selected from the group consisting of trichlorodiphenyl, tetrachlorodiphenyl, pentachlorodiphenyl, hexachlorodiphenyl, polychlorotriphenyl, pentachlorodiphenyl oxide, pentachlorodiphenyl benzoate, hexachlorodiphenyl methane, and pentachlorodiphenyl ketone.

The present invention relates to an electric contact grease which has particular application in power switches of electrical machines and apparatuses.

Usual electric contacts of, for example, television and radio are subjected to contact failure and contact welding and are responsible for troubles such as sound noise, picture failure, impossibility of contact opening and the like.

These troubles are prevented to some extent by using existing electric contact greases. However, such use has not been completely satisfactory due to the complicated nature of the phenomenon of the electric contact. Contact failures are usually caused by oxidation, sulfation, and wear of contact metal surfaces and sludge formed by oxidation, polymerization, and burning of the grease itself.

Excellent contact greases to remove such troubles have been long desired especially in the case of base metal contact such as copper or brass which are easily subjected to contact failures.

Therefore the role of contact grease is to prevent oxidation, sulfation and wear of contact metals and thereby to stabilize the electric contact resistance and to prevent noise and at the same time, prevent contact welding by restraining temperature rise of the electric contacts.

An object of the present invention is to provide a contact grease capable of suppressing a rise in the electric contact resistance of an electric contact.

A further object of the present invention is to provide a contact grease which prevents an electric contact from wearing.

Another object of the present invention is to provide a contact grease useful for use in an electric contact formed by copper, brass, phosphorous bronze, beryllium copper and nickel silver.

These and other objects of the present invention will be apparent upon consideration of the following detailed description.

A contact grease according to the present invention consists essentially of a major amount of paraffinic mineral

oil, 10 to 20 percent by weight of, as a thickening agent, a mixture of metallic soaps and 7 to 15 percent by weight of at least one member selected from the group consisting of chlorinated aromatic hydrocarbon and its derivatives.

- 5 Said mixture of metallic soaps consists essentially of 40 to 65 percent by weight of barium soap, 25 to 40 percent by weight of lithium soap and 10 to 20 percent by weight of aluminum soap in accordance with the present invention. The novel contact grease according to the present invention prevents an electric contact from failing, and welding which ensures a satisfactory contacting action for a longer time period especially when applied to an electric contact made of corrodible metal such as copper, brass, phosphorous bronze, beryllium copper and nickel silver. Antirust agent and/or antioxidant are preferably added to the composition of the grease.

A contact grease according to the present invention can employ chlorinated aromatic hydrocarbon or its derivatives having a boiling point higher than 300° C. Chlorinated aromatic hydrocarbon or its derivatives serve to prevent temperature rise and contact wear by restraining burning of grease by arcing and at the same time by acting as lubricating agent. A better result can be obtained by employing at least one member selected from the

- 20 group consisting of trichlorodiphenyl, tetrachlorodiphenyl, pentachlorodiphenyl, hexachlorodiphenyl, polychlorotriphenyl, pentachlorodiphenyl oxide, pentachlorophenyl benzoate, hexachlorodiphenyl methane, and pentachlorodiphenyl ketone. Among those members, trichlorodiphenyl, tetrachlorodiphenyl, hexachlorodiphenyl, polychlorotriphenyl achieve the best results in accordance with the present invention.

If the chlorinated aromatic hydrocarbon or derivative thereof is present in an amount lower than about 7% by weight, the temperature rise of contact goes higher, while an amount greater than about 15% by weight makes it difficult to produce a contact grease having a good homogeneity.

- 35 The paraffinic mineral oil defined herein includes pure paraffinic mineral oil as well as impure paraffinic mineral oil having incorporated therein a small amount, for example up to 30% by weight of aromatic and/or naphthenic mineral oil. It is preferable that the paraffinic mineral oil has a viscosity of 40 to 180 cst. (at 37.8° C.) and an aniline point higher than 90 in the ASTM D611-55T (American Society for Testing Materials).

One can employ barium soap, lithium soap and aluminum soap including those containing an aliphatic fatty acid radical. Their chemical formulae are expressed by Ba(RCOO)<sub>2</sub>, Li(RCOO) and Al(RCOO)<sub>3</sub>, respectively where R is an alkyl radical. However, these chemical formulae should not be construed to define only pure substances, but include impure substances incorporated with unavoidable impurities. For example, Al(RCOO)<sub>3</sub> commercially available includes Al(OH)(RCOO)<sub>2</sub> in an amount of less than 20 percent by weight and is operable for production of a contact grease according to the present invention. It is preferable that the R in the chemical formulae contains 12 to 20 carbon atoms. The most preferable barium soap, lithium soap and aluminum soap is one which includes a stearic acid radical.

The content of free fatty acid of these metallic soaps is desirably small, preferably lower than 2 percent by weight.

- 50 In connection with the weight percent of the mixture of metallic soaps, the following is noted: The barium soap in an amount higher than 65 percent by weight increases the electric contact resistance and the barium soap in an amount lower than 40 percent by weight impairs the resistance to welding of electric contact; the lithium soap in an amount lower than 25 percent by weight increases the electric contact resistance and the lithium soap in an amount higher than 40 percent by weight impairs the re-

sistance to the welding; and the aluminum soap in an amount higher than 20 percent by weight produces a contact grease which has a low pour point and is inferior in the resistance to heat and the aluminum soap in an amount lower than 10 percent by weight results in a contact grease which is poor in homogeneity.

When the amount of the mixture of the metallic soaps in the grease is less than about 10 percent by weight, the resultant contact grease is too soft to hold its shape as it is. On the other hand, an amount of the mixture higher than about 20 percent by weight results in a contact grease which is too hard.

A contact grease according to the present invention can be improved by using an antioxidant and/or a rust inhibitor. The preferable antioxidants are

n-butyl-p-aminophenol,  
di-sec-butyl-p-phenylenediamine,  
4,4'-tetramethyl-diaminodiphenyl methane,  
 $\alpha$ -naphthylamine,  
n,n'-di-salicylidene-1,2-propylenediamine,  
2,6-di-tert-butyl phenol,  
2,4-dimethyl-6-tert-butyl phenol,  
2,6-di-tert-butyl-p-cresol,  
4,4'-methylenebis(2,6-di-tert-butyl phenol),  
2,2'-methylenebis(4-methyl-6-tert-butyl phenol),  
4,4'-butyldene bis(3-methyl-6-tert-butyl phenol).

The preferable rust inhibitor is sorbitan mono-oleate, salt of dinonyl naphthalene sulphonate,  $\alpha$ -(2-carboxy phenoxy) stearic acid. The amount of the antioxidant is preferably 0.01 to about 3 percent by weight, that is 0.01 to 3 percent by weight of the antioxidant and about 97 to 99.99 percent by weight of the contact grease. The amount of the rust inhibitor is 0.01 to about 4 percent by weight of the rust inhibitor and about 96 to 99.99 percent by weight of the contact grease.

A mixture of the paraffinic mineral oil, the mixture of the metallic soaps, the chlorinated aromatic hydrocarbon or its derivatives with or without antioxidant and rust inhibitor is heated at 200-250° C., to make a homogeneous liquid and then cooled to room temperature. The cooled mixture is milled by a usual method, e.g. employing three roll mills, and is subjected to the removal of airfoams at a reduced pressure.

The resulting greases are smooth and buttery in texture and have excellent mechanical and thermal stability.

The invention is illustrated in the ensuing examples which are for the purpose of illustration and are not considered to be wholly definitive with respect to scope or conditions. In the examples "g." represents grams.

#### EXAMPLE 1

A mixture of 74.7 g. of paraffinic mineral oil having viscosity of 60 cst. at 37.8° C. and aniline point of 11.7° C., 8 g. of barium stearate (M.P. 235° C.), 5 g. of lithium stearate (M.P. 221° C.), 2 g. of aluminum stearate (M.P. 112° C.), 10 g. of polychlorotriphenyl, 0.1 g. of 4,4'-tetramethyl diamino diphenyl methane and 0.2 g. of sorbitan monooleate is stirred and heated at 230 to 240° C.

After being homogenized the mixture is poured into a dish and cooled to room temperature, milled with a three roll mill, and then the remaining foam of the grease is removed under reduced pressure. The resulting grease is stable and has an ASTM penetration of 332 and a pour point of 120° C. The grease is applied to an electric contact made of copper and brass. The grease action is shown in Example No. 1 of the table.

#### EXAMPLE 2

A mixture of 70.5 g. of paraffinic mineral oil having viscosity of about 50 cst. at 37.8° C. and aniline point of 102.7° C., 10 g. of barium stearate (M.P. 235° C.), 7 g. of lithium stearate, 4 g. of aluminum stearate, 8 g. of polychlorotriphenyl, and 0.5 g. of 2,6-di-tert-butyl phenol is heated at 235 to 245° C. After being homogenized the mixture is cooled, milled and treated in a manner similar

to that of Example 1. The testing result carried out similarly to Example 1 is shown in the table.

#### EXAMPLE 3

5 A mixture of 73.8 g. of paraffinic mineral oil having viscosity of 120 cst. at 37.8° C. and aniline point of 114.9° C., 6 g. of barium stearate (M.P. 250° C.), 4 g. of lithium stearate, 14 g. of polychlorotriphenyl, 0.2 g. of Na salt of dinonyl naphthalene sulphonate is stirred and heated at 10 about 250° C. The clear fluid solution is treated in a way similar to that of Example 1. The testing result carried out similarly to Example 1 is shown in the table.

#### EXAMPLE 4

15 A mixture of 75.4 g. of paraffinic mineral oil having viscosity of 80 cst. at 37.8° C. and aniline point of 114.0° C., 7 g. of barium stearate, 5 g. of lithium laurate (M.P. 219° C.), 1.5 g. of aluminum stearate, 8 g. of hexachloro diphenyl, 0.1 g. of tetra base and 3 g. of sorbitan monooleate is heated in a beaker until its temperature reaches about 240° C. The resulting mixture is treated in a way similar to that of Example 1. The testing result carried out similarly to Example 1 is shown in the table.

#### EXAMPLE 5

20 A mixture of 72.9 g. of paraffinic mineral oil having viscosity of 60 cst. at 37.8° C. and aniline point of 111.7° C., 10 g. of barium stearate, 5 g. of lithium laurate (M.P. 219° C.), 3 g. of aluminum stearate and 9.1 g. of tetrachloro diphenyl is stirred and heated in a beaker until its temperature reached about 250° C. The resulting mixture is treated in a way similar to that of Example 1. The testing result carried out similarly to Example 1 is shown in the table.

#### EXAMPLE 6

25 A mixture of 70.9 g. of paraffinic mineral oil having viscosity of 80 cst. at 37.8° C. and aniline point of 114.0° C., 9 g. of barium stearate (M.P. 240° C.), 6 g. of lithium laurate (M.P. 219° C.), 2 g. of aluminum stearate (M.P. 110° C.), 12 g. of polychlorotriphenyl and 0.1 g. of tetra base is stirred and heated in a beaker and treated in a way similar to that of Example 1. The testing result carried out similarly to Example 1 is shown in the table.

#### EXAMPLE 7

30 A mixture of 69.8 g. of paraffinic mineral oil having viscosity of 78.2 cst. at 37.8° C. and aniline point of 104.2° C., 10 g. of barium stearate, 6 g. of lithium stearate, 2 g. of aluminum stearate, 11 g. of polychlorotriphenyl, 0.2 g. of tetra base and 1 g. of span 80 is stirred and heated in a beaker and treated in a way similar to that of Example 1. The testing result carried out similarly to Example 1 is shown in the table. Span 80, in the above 35 example, is sorbitan monooleate.

#### EXAMPLE 8

35 A mixture of 73.7 g. of paraffinic mineral oil having viscosity of 80 cst. at 37.8° C. and aniline point of 114.0° C., 8 g. of barium stearate, 6 g. of lithium stearate, 2.2 g. of aluminum stearate, 10 g. of polychlorotriphenyl and 0.1 g. of tetra base is stirred and heated in a beaker and treated in a way similar to that of Example 1. The testing result carried out similarly to Example 1 is shown in the table.

#### EXAMPLE 9

40 A mixture of 76.5 g. of paraffinic mineral oil having viscosity of 120 cst. at 37.8° C. and aniline point of 114.9° C., 8 g. of barium stearate, 4 g. of lithium stearate, 1.5 g. of aluminum stearate, 9 g. of hexachloro diphenyl, and 1.0 g. of 2,2'-methylene bis(4-methyl-6-tert-butyl phenol) is stirred and heated in a beaker and treated in a way similar to that of Example 1. The testing result carried 45 out similarly to Example 1 is shown in the table.

C., 7 g. of barium stearate, 6 g. of lithium stearate, 2 g. of aluminum stearate, 11 g. of polychlorotriphenyl, and 0.2 g. of tetra base is stirred and heated in a beaker and treated in a way similar to that of Example 1. The testing

In the foregoing examples, tetra base is 4,4'-tetramethyl diamino diphenyl methane.

TABLE

| Contact metal                              | Example Number  |         |         |         |         |                   |                   |                   |                   |                   |
|--------------------------------------------|-----------------|---------|---------|---------|---------|-------------------|-------------------|-------------------|-------------------|-------------------|
|                                            | Combination of— |         |         |         |         |                   |                   |                   |                   |                   |
|                                            | Copper          | Copper  | Copper  | Copper  | Copper  | Copper            | Copper            | Copper            | Copper            | Copper            |
| Brass                                      | Brass           | Brass   | Brass   | Brass   | Brass   | Beryllium, Copper | Beryllium, Copper | Beryllium, Copper | Beryllium, Copper | Beryllium, Copper |
| 200                                        | 200             | 200     | 200     | 200     | 200     | 300               | 300               | 300               | 300               | 300               |
| 30                                         | 30              | 30      | 30      | 30      | 30      | 50                | 50                | 50                | 50                | 50                |
| 100                                        | 100             | 100     | 100     | 100     | 100     | 100               | 100               | 100               | 100               | 100               |
| 100                                        | 100             | 100     | 100     | 100     | 100     | 100               | 100               | 100               | 100               | 100               |
| (1)                                        | (1)             | (1)     | (1)     | (1)     | (1)     | (1)               | (1)               | (1)               | (1)               | (1)               |
| 8                                          | 7               | 5       | 4       | 5       | 3       | 4                 | 5                 | 5                 | 8                 | 7                 |
| 18                                         | 24              | 34      | 25      | 29      | 18      | 29                | 29                | 22                | 16                | 25                |
| 39                                         | 55              | 49      | 32      | 35      | 42      | 15                | 48                | 39                | 48                | 58                |
| 28                                         | 79              | 81      | 44      | 162     | 78      | 22                | 75                | 69                | 83                | 2,310             |
| Number of on-off operations until welding. |                 | >50,000 | >50,000 | >50,000 | >50,000 | >50,000           | >50,000           | >50,000           | >50,000           | >50,000           |

<sup>1</sup>Rush, 30; normal, 4. <sup>2</sup>Lamp load; normal, 4.

What is claimed is:

1. A contact grease consisting essentially of  
(a) a major amount of paraffinic mineral oil;  
(b) 10 to 20 percent by weight of, as a thickening agent,  
a mixture of metallic soaps, said mixture of metallic  
soaps consists essentially of

(i) 40 to 65 percent by weight of barium soaps;  
(ii) 25 to 40 percent by weight of lithium soap, and;  
(iii) 10 to 20 percent by weight of aluminum soap;  
and

(c) 7 to 15 percent by weight of at least one member  
selected from the group consisting of trichlorodiphenyl,  
tetrachlorodiphenyl, pentachlorodiphenyl,  
hexachlorodiphenyl, polychlorotriphenyl, pentachloro-  
rophenyl oxide, pentachlorophenyl benzoate, hexa-  
chlorodiphenyl methane, and pentachlorodiphenyl  
ketone.

2. A contact grease of claim 1, wherein barium soap,  
lithium soap and aluminum soap are essentially  
20 Ba(RCOO)<sub>2</sub>, Li(RCOO), Al(RCOO)<sub>3</sub>, respectively,  
wherein R represents alkyl radical containing from 12 to  
20 of carbon atoms.

25 3. A contact grease defined by claim 1 further including  
0.01 to 3.0 percent by weight of an antioxidant selected  
from the group consisting of n-butyl-p-aminophenol,  
di-sec-butyl-p-phenylenediamine, 4,4'-tetra-methyl-diaminodiphenyl-methane,  $\alpha$ -naphthylamine, n,n'-di-  
30 salicylidene-1,2-propylenediamine, 2,6-di-tert-butyl-phenol,  
2,4-dimethyl-6-tert-butyl-phenol, 2,6-di-tert-butyl-p-  
cresol, 4,4'-methylene-bis-(2,6-di-tert-butyl-phenol), 2,2'-  
methylenebis(4-methyl-6-tert-butyl-phenol), 4,4'-butyl-  
idene-bis-(2-methyl-6-tert-butyl-phenol).

35 4. A contact grease defined by claim 1, further including  
0.01 to 4 percent by weight of an antirust agent selected  
from the group consisting of sorbitan monooleate,  
salt of dinonyl naphthalene sulphonate, and  $\alpha$ -(2-carboxy-  
phenoxy)-stearic acid.

#### References Cited

##### UNITED STATES PATENTS

2,375,485 5/1945 Morgan et al. ----- 252—36  
2,420,902 5/1947 Morway et al. ----- 252—36

40 DANIEL E. WYMAN, Primary Examiner

45 I. VAUGHN, Assistant Examiner

U.S. Cl. X.R.

252—35, 36, 39, 521